

# UNITED STATES PATENT OFFICE.

ROBERT S. MILLER, OF WILMINGTON, DELAWARE, ASSIGNOR OF ONE-HALF  
TO JAMES WILBUR CARRIER, OF SAME PLACE.

## BOILER AND PIPE COVERING.

SPECIFICATION forming part of Letters Patent No. 465,718, dated December 22, 1891.

Application filed August 5, 1891. Serial No. 401,773. (Specimens.)

*To all whom it may concern:*

Be it known that I, ROBERT S. MILLER, residing at Wilmington, New Castle county, State of Delaware, have invented a new and useful Improvement in Boiler and Pipe Coverings, of which the following is a specification.

My invention consists in an improved composition to form an elastic boiler and steam-pipe covering.

The following are the ingredients for making five barrels of the covering: refined or washed kaolin, one and one-half barrels; cow or goat hair, one-half bushel; asbestos fiber, two bushels; feldspar, three pecks; plaster-of-paris, twelve quarts; rag pulp, one barrel; ground cork, ten pounds; sal-ammoniac, one pound. Add sufficient water to make a mortar and mix thoroughly.

20 The composition is put on in two coats. For the first coat for boiler and steam-pipe covering the plaster-of-paris is omitted, and the amount of asbestos is increased and of rag pulp diminished, depending on the amount

25 of heat. When the composition is to be spread on canvas for covering pipes, the kaolin is reduced one-half for both first and second coatings. Ordinarily, however, the composition is used as per formula given, and is applied 30 with a trowel like plaster, the boiler or pipe being first covered with wire-netting, into which the composition penetrates and by which it is retained in a manner similar to that by which laths holds the plaster.

35 The kaolin, hair, and asbestos are common ingredients in boiler-coverings, and for these no special claims are made.

The following are the distinctive features 40 of my invention: The use of sal-ammoniac neutralizes grease or oil and makes the covering adhere to greasy iron. It also destroys all bad odor arising from the covering coming in contact with fire or steam heated surfaces. The feldspar gives the composition

45 a stiff and sticky nature and causes the covering to adhere to the iron without the use of straps. It is also one of the ingredients that help to make the covering elastic. The plaster-of-paris is not put in as a cement, as the covering will hold together without it, and an ex-

cess of plaster-of-paris would make the covering so hard that it would crack with the expansion and contraction of the boiler. Either plaster-of-paris or kaolin when used alone as an outside coating or finish for boiler and steam pipe coverings will crack; but when the plaster-of-paris, feldspar, and kaolin are thoroughly mixed together and mixed with the other ingredients of the covering they give the covering a smooth and water-proof 60 finish, which will take a high polish by rubbing with a cloth, and also make the covering elastic so that it will expand and contract with the iron without cracking. This smooth glossy water-proof finish prevents cracks and 65 constitutes one of the principal advantages of this covering.

The following are some of the advantages claimed for the composition taken as a whole:

First, it is fire-proof, (cannot be made to 70 burn.)

Second, being elastic and expanding and contracting with the boiler, it is free from cracks.

Third, it never falls off and clings to all 75 work without straps, and not being made of perishable materials is claimed to be the most durable of coverings.

Fourth, it is an anti-rust covering, containing no ingredients that will corrode the iron 80 and prevents the formation of rust.

Fifth, it is an odorless covering, which is a great advantage in a dwelling-house.

Sixth, it is water-proof.

Seventh, it is one of the best non-conductors of heat.

Eighth, the composition takes a high polish and presents a beautiful appearance.

Hydraulic cement or lime may be used as a substitute for the plaster-of-paris, and in 90 this case would be the equivalent thereof; but the cement or lime must not be used in excess, as then the covering would not be elastic.

Cements have been used in boiler-coverings before; but they were used for an entirely 95 different purpose—namely, to hold the covering together, and such coverings crack.

This water-proof finish on my covering saves the expense of putting on canvas or other similar outside coverings, which are not wa- 100

ter-proof, and which soon become dirty and cannot well be cleaned, whereas my covering can be washed as often as desired.

Having thus described my invention, what I claim is—

The composition herein described, consisting of kaolin, hair, asbestos, feldspar, plaster-

of-paris or its described equivalent, rag pulp, ground cork, and sal-ammoniac in or about the proportions described.

ROBERT S. MILLER.

Witnesses:

J. W. CARRIER,  
MARGARET MILLER.